

# UNITED STATES PATENT OFFICE.

EDWARD D. GLEASON, OF NEW YORK, N. Y., ASSIGNOR TO PLASTIC METAL COMPANY,  
OF NEW YORK, N. Y., A CORPORATION OF NEW YORK.

## PROCESS OF MAKING LEAD-COPPER COMPOSITIONS.

1,077,700.

Specification of Letters Patent.

Patented Nov. 4, 1913.

No Drawing. Original application filed March 7, 1913, Serial No. 752,601. Divided and this application filed March 31, 1913. Serial No. 757,860.

*To all whom it may concern:*

Be it known that I, EDWARD D. GLEASON, a citizen of the United States, residing in Brooklyn, in the county of Kings, city and

5 State of New York, have invented a certain new and useful Improvement in Processes of Making Lead-Copper Compositions, whereof the following is a specification.

10 This application is a division of my application Serial #752,601, filed March 7, 1913 for Letters Patent of the United States for improvement in lead-copper compositions.

15 My invention relates to plastic compositions including lead and copper, and lead-copper and tin, which may be advantageously used in the manufacture of bearings for shafts, etc.

20 It is an object of my invention to provide such compositions free from "lead sweats" and segregation, which are defects usually found in such compositions due to lack of affinity of the lead for the copper or copper and tin, and the high specific gravity and 25 low melting point of lead, for, at best, such compositions are but mechanical mixtures wherein copper is held in a finely divided state in a matrix of lead.

Another object of my invention is to provide 30 such compositions including a given percentage of copper but of different degrees of hardness.

35 The effect of my improvement is to provide a composition which is homogeneous in that the copper therein is comminuted to the greatest possible extent and equally distributed throughout the mass of the composition. I have discovered that the effect aforesaid is attained by adding to the molten 40 copper, in the process of making such compositions, a non-metallic derivative of the other metal, capable of increasing the miscibility of copper with that metal, to wit, lead sulfid, and particularly the native 45 lead sulfid, galena. For instance, I fuse 50 pounds of copper and add thereto 5 pounds of galena and then gradually add, to said mixture, 45 pounds of lead. The fused mix-

ture is then poured into pig, ingot or other suitable molds, and, when congealed, fracture thereof shows that the cast metal is homogeneous.

50 Harder alloys may be formed by taking 50 pounds of copper, 10 pounds of galena and 40 pounds of lead or 45 pounds of copper, 10 pounds of galena and 45 pounds of lead; said ingredients being mixed as in the first instance above described. 55

As above indicated, the use of galena is effective for the purpose described when used in alloys containing tin. For instance, I take 60 parts copper, 30 parts lead, 5 parts galena and 5 parts tin, or, 55 parts copper, 60 35 parts lead, 5 parts galena and 5 parts tin. However, such alloys including tin form the subject matter of my application Serial #752,600, filed March 7, 1913 for Letters Patent of the United States. 65

I do not desire to limit myself to the precise methods of procedure or proportions herein set forth as it is obvious that various modifications may be made therein without departing from my invention as defined in 70 the appended claims.

I claim:—

1. A process of making a composition containing copper and lead which consists in fusing said metals with lead sulfid and 75 thereby increasing the miscibility of said metals.

2. A process of making a composition which consists in fusing lead sulfid with copper and then adding lead thereto and 80 fusing the mixture.

3. A process of making a composition which consists in fusing with copper a non-metallic derivative of another metal, capable of increasing the miscibility of copper with 85 that metal, and then adding the other metal thereto and fusing the mixture.

4. The process of making a composition containing copper and another metal which consists in fusing with the copper a sulfid 90 of the other metal, and then mixing the other metal therewith.

5. A process of making a composition

containing copper and another metal which consists in fusing therewith a non-metallic derivative of the other metal, capable of increasing the miscibility of copper with that metal.

5 In testimony whereof, I have hereunto

signed my name at Brooklyn, New York,  
this twenty-eighth day of March, 1913.

EDWARD D. GLEASON.

Witnesses:

BENJAMIN ZEKOWSKI,  
SIEGMUND ZEKOWSKI.